

Patented May 19, 1936

2,041,655

# UNITED STATES PATENT OFFICE

2,041,655

## WOOD TREATING PREPARATION

Gilbert Gunn, Pollokshaws, Scotland, assignor to  
Celicure Corporation of America, Worcester,  
Mass., a corporation of Massachusetts

No Drawing. Application November 16, 1934,  
Serial No. 753,306. In Great Britain November  
24, 1933

4 Claims. (Cl. 134—78.6)

This invention relates to wood treating preparations and has for one of its objects a dry preparation containing all the necessary ingredients for treating wood to preserve it from rot and attack by insects, except the water required to dissolve the ingredients at the time the wood is impregnated therewith.

Another object is to provide a preparation which contains a fireproofing ingredient as well as preservative constituents.

Heretofore when wood preservative substances, like soluble dichromates and copper salts, have been used as wood preservatives they have been acidified by acetic acid in liquid form, usually in the form of pyroligneous acid, the function of which is by acidifying the mixture to intensify the oxidizing action of the dichromate on the lignose and other constituents of the wood and to prevent the separation of substantially insoluble basic copper chromate before the wood has been impregnated.

Acetic acid, either in pure form or as pyroligneous acid, is a liquid and has a corrosive action on many materials. It is, therefore, troublesome and expensive to ship. The quantity of acetic acid required is not a large part of the total preparation, but the fact that acetic acid is a corrosive liquid necessitates either the separate shipment of the dichromate and copper salt, on the one hand, and the acetic acid on the other or the use of liquid-tight non-corrosive containers for the mixture of all three ingredients.

According to the present invention, therefore, a dry acidifying material, is used so that all of the ingredients may be shipped in dry form, advantageously mixed so that all that is required is to add water and apply.

The acidifying material is a salt which, when a solution thereof is brought into contact with the wood, will yield an acid. Such salts are chromium or aluminum acetate or the formate, butyrate and many other salts of such metals.

The action of such material is apparently due to hydrolysis, followed by a progressive reaction between the basic part of the compound and the constituents of the wood which leaves behind the acid in a free state to intensify the oxidizing action of the dichromate and prevent premature separation of substantially insoluble basic copper chromate.

As the action of the dichromate part of the preparation is to oxidize certain constituents of the wood, I prefer not to use salts of reducing acids, such as oxalic, tartaric or citric acids.

Further, for uses where corrosion of metal parts is to be avoided, it is preferable to use a hydrolyzable salt of a volatile acid like acetic acid instead of a solid, non-volatile acid, like malic or lactic acid. A volatile acid will evaporate after it has aided the action of the di-

chromate on the wood and not remain to act as a corrosive agent on iron, steel or other parts embedded in or in contact with the wood.

I have also found that salts of volatile relatively weak acids, like acetic acid, have marked advantages over volatile strong acids like hydrochloric acid. Likewise, salts of sulphuric and nitric acid are not as suitable as salts of acids of the acetic acid type.

The hydrolyzable salt may be formed from any one of a number of metals forming very weak bases, like chromium, iron, copper and aluminum.

Various soluble dichromates may be used, although the cheapest and hence most advantageous ones are sodium and potassium dichromates. The former is highly deliquescent and has such a strong affinity for water that it will extract water of crystallization from copper sulphate crystals ( $\text{CuSO}_4 \cdot 5\text{H}_2\text{O}$ ) and go into solution in the water so extracted. The result is a paste, and, if the mixture contains chromium acetate, the latter will dissociate prematurely and give off acetic acid.

The production of a paste may be avoided by using either potassium or ammonium dichromate, which is much less deliquescent, or partially or wholly dehydrated copper sulphate or some other soluble copper salt, like the chloride, which does not contain sufficient water of crystallization to permit the mixture to become pasty.

Small percentages of chemicals which increase toxicity but do not corrode metals may be added, for example:— boric acid  $\text{H}_3\text{BO}_3$ : cadmium chloride  $\text{CdCl}_2 \cdot 2\text{H}_2\text{O}$  and others.

A suitable formula for my preparation in the dry state is the following:

|                                                                                              | Per cent |
|----------------------------------------------------------------------------------------------|----------|
| Potassium dichromate ( $\text{K}_2\text{Cr}_2\text{O}_7$ )                                   | 48.15    |
| Copper sulphate ( $\text{CuSO}_4 \cdot 5\text{H}_2\text{O}$ )                                | 43.00    |
| Chromium acetate ( $\text{Cr}(\text{C}_2\text{H}_3\text{O}_2)_3 \cdot 3\text{H}_2\text{O}$ ) | 4.55     |
| Boric acid ( $\text{H}_3\text{BO}_3$ )                                                       | 4.30     |
|                                                                                              | 100.00   |

0.93 or say 1 lb. of the above preparation per U. S. gallon will give a solution (full strength) for brushing or spraying of the following composition:

|                      | Per cent |
|----------------------|----------|
| Potassium dichromate | 5.60     |
| Copper sulphate      | 5.00     |
| Chromium acetate     | 0.53     |
| Boric acid           | 0.50     |
| Water                | 88.37    |
|                      | 100.00   |

The boric acid is not an essential constituent and may be omitted if desired. For the treatment of timber under pressure one half the foregoing per-

percentages in solution of the dichromate and copper sulphate may be used but it is advisable to retain the original percentages of chromous acetate and boric acid.

5 I have found that wood which has been treated with a slightly acid aqueous solution of a soluble dichromate and a soluble copper salt is rendered substantially impenetrable to salt and other solutions. Hence wood so treated cannot be subsequently impregnated with solutions of fire-proofing substances. I have found that impregnation with certain of such substances can take place if they are mixed with the dichromate mixture.

10 I have found however if fireproofing material is mixed with the dichromate mixture to penetrate the wood with the latter, the impregnation of the wood with the preserving agents is interfered with in the case of many of the well known 15 fireproofing agents due to insoluble precipitates.

I have found however that boric acid can be used very satisfactorily in admixture with soluble dichromate and copper salts.

20 A suitable formula for my fireproofing composition is the following:

|                                                   | Per cent |
|---------------------------------------------------|----------|
| Potassium dichromate ( $K_2Cr_2O_7$ )             | 34       |
| Copper sulphate ( $CuSO_4 \cdot 5H_2O$ )          | 30       |
| Chromium acetate ( $Cr(C_2H_3O_2)_3 \cdot H_2O$ ) | 6        |
| 30 Boric acid ( $H_3BO_3$ )                       | 30       |
|                                                   | 100      |

25 Full strength of solution is obtained by adding 1 lb. of the above dry mixture to each U. S. gallon water.

The strength of the solution may be varied widely depending on the hardness and other qualities of the wood or the like.

30 It is advisable for many reasons to dissolve the mixture in hot water. One reason is, that chromium acetate reacts with the constituents of wood very slowly in cold water. Another reason is that boric acid is only sparingly soluble in cold water, so that when concentrated solutions are required the boric acid will not go into solution at full strength below 100° C.

35 The proportions given in the above formula are of course, merely illustrative of many that may be used satisfactorily. I have found, however, that greater latitude may be allowed in the proportion of acetate and/or boric acid to the other constituents than in the proportion of dichromate relatively to copper. Ordinarily the percentage of 40 chromium acetate should be between 0.5 and 10% of the dry mixture to advantage between 2 and 5%.

45 The boric acid content may vary widely according to the nature of the wood and the degree of fireproofing desired. Usually the percentage of boric acid should not be much below 5 or better 10% or the fireproofing qualities will be seriously impaired. Of course, if the solution is diluted to any great extent and it is desired to 55 obtain the maximum possible fireproofing, the proportion of boric acid may be increased correspondingly.

60 The proportion of acidifying material used may also be increased to advantage, with dilution of the solution as the action of the acid is weakened

by its dilution, and the weaker the solution of dichromate the more it needs acid stimulation.

65 In place of boric acid I may use as a fireproofing material phosphoric acid and/or a phosphate and sufficient acidifying material to prevent the precipitation of insoluble copper (or chromium) phosphate prior to impregnation of the wood. After the wood has been impregnated, precipitation of insoluble phosphates takes place due to the volatilization of the acid. The insoluble phosphates left behind are fire-proofing materials and being insoluble are not leached out by rain, etc.

70 In view of the need of acid to prevent premature precipitation of copper phosphate an acid phosphate such as mono-ammonium phosphate ( $(NH_4)_2HPO_4$ ) may be used. However, as neither phosphoric acid nor sulphuric acid are volatile, it may be desirable to use the tri-basic phosphate ( $(NH_4)_3PO_4$ ) and secure the desired acidity by the use of more acetic acid or other volatile acid 75 than would otherwise be necessary. Other phosphates than ammonium, such as sodium, potassium or even copper or zinc may be used.

80 When other phosphates than copper are used it is advisable to use additional copper or zinc sulphate to react with the phosphate added and thus avoid upsetting the relationship between the dichromate and copper salt necessary for preservation purposes.

85 When mono-ammonium phosphate is used in place of boric acid, a suitable proportion is an amount equal (by weight) to the boric acid in the foregoing formula, with an equal amount of additional copper or zinc sulphate and chromium acetate.

90 The above proportions may be varied widely, the chief requirement being that there should be sufficient acid to keep the phosphates in solution during the impregnation period.

If desired the composition may include both boric acid and/or borax as well as phosphate.

95 I may use ammonium sulphate in small quantity if found necessary, but as in large quantity it tends to keep wood treated therewith moist indefinitely, it is not ordinarily as suitable as either boric acid or phosphates.

What is claimed is:

1. A new wood preservative in dry form, comprising a soluble dichromate, a soluble copper salt and a non-reducing salt of a weak volatile aliphatic acid and a base capable of reacting with the wood to liberate the acid part of such salt, the proportion of the last named salt being less than either of the first two salts.

2. A new wood preservative in dry form, comprising as major constituents a soluble dichromate, a soluble copper salt and a fire-proofing material of the group consisting of boric acid, borates and phosphates, and as a minor constituent a non-reducing salt of a weak volatile aliphatic acid and a base capable of reacting with the wood to liberate the acid part of such salt.

3. A wood preservative as in claim 1, in which the non-reducing salt is a salt of a metal of the group consisting of chromium, iron, copper and aluminum.

4. A wood preservative as in claim 1, in which the non-reducing salt is one of the group consisting of chromium and aluminum acetates.